

Patented Nov. 23, 1926.

1,608,250

# UNITED STATES PATENT OFFICE.

ROBERT JAY SHOEMAKER, OF CHICAGO, ILLINOIS, ASSIGNOR TO LEADIZING COMPANY, OF CHICAGO, ILLINOIS, A CORPORATION OF ILLINOIS.

## PLATING METHOD.

No Drawing.

Application filed July 13, 1923. Serial No. 651,415.

My invention relates to a novel method of coating or plating metal articles or bodies, particularly of iron or steel, with a plating metal or metals.

5 The method consists in first immersing the article in a solution of a salt of a suitable plating metal from which the metal will be deposited in an adherent film or coating on the article treated, or in bringing the 10 article into contact, by immersion or otherwise, with a body of plating metal in a molten state to produce a like film or coating thereon, and then producing a further deposition either of the same or of another plating metal by electrolytic action.

The method is of particular utility in the plating of iron or steel articles with lead. When an attempt is made to plate an iron or steel article with lead by electrolysis difficulty is experienced in obtaining a coating which will be dense, smooth and permanently adherent. Due probably to the necessary lack of concentration of the electrolyte and the tendency of the same to react 25 chemically with the iron the deposit of lead is spongy and uneven. A dense coating of lead can be obtained without the use of an electric current by means of a highly concentrated solution of lead acetate, or by the 30 immersion of the article in a lead bath, but in such case the coating will be thinner than is sometimes desirable. For example, it is hardly feasible to obtain in this way a coating of more than one and a half to two 35 ounces per square foot.

I have discovered, however, that if the article is first dipped into a solution of lead acetate, for example, or after suitable fluxing into a molten bath of lead (the former 40 expedient being preferable for reasons of economy) and is then treated electrolytically a very dense, smooth, adherent plating may be obtained of any thickness desired. For example, the lead coating may 45 be built up to a thickness of from six to eight ounces per square foot.

The first lead plating operation may also be advantageously combined with a subsequent electro-plating of the article with copper or some metal other than lead, for example, with copper, tin, nickel or silver. In the case of nickel or tin plating the intermediate lead plating prevents rusting through. By first coating an article with 50 lead and then with copper a good substitute

for solid copper may be obtained at a very low cost. For silver plating the underlying lead coating decreases cost by making possible a thinner plating of the plating metal.

In the place of lead for the first coating when the hot dipping method is employed, it is possible to use mixtures of lead and tin, or lead, tin and antimony, or tin alone or mixed with a small amount of antimony.

60 The first plating operation may be accomplished by either of the following two methods:

(1) The article is first cleaned in the usual manner by means of a suitable acid 70 for the purpose of removing traces of rust or grease. It is then immersed in a concentrated water solution of lead acetate and acetic acid. The solution should contain at least 35% by weight of lead acetate although, 75 to get the best results, the lead acetate content should be 40% to 50%. The acetic acid should not be less than 5%. The solution is heated. Otherwise the action will be extremely slow. Preferably it is maintained 80 at a temperature of from 160° to 180° Fahrenheit. As the solution becomes impoverished it may be built up by adding lead acetate crystals, water and acetic acid. The article is then withdrawn from the solution 85 and washed with water.

(2) In place of the treatment just described the article, after being cleaned with an acid and covered with a flux may be immersed in a bath of molten lead. Preferably 90 the flux is composed of 80% by weight of zinc chloride and 20% by weight of common salt and is supported in a confined area on the surface of the lead bath. The article is passed through the flux into the lead 95 bath which latter is maintained at a temperature of approximately 700° Fahrenheit. After removal of the article from the bath it is washed.

With either of the above methods the 100 article is covered with a dense adherent film or coating of lead which, however, may be thinner than is desirable.

Assuming that a thicker coating of lead is required, the article is then introduced into 105 an electrolytic cell containing a 10% water solution of lead acetate, or in place of the lead acetate solution a 10% solution of lead silica-fluoride. Preferably I add to the electrolyte a soluble distillate of an organic 110

carbohydrate such for example, as a water soluble product of the dry distillate of wood, known commonly as wood tar. The organic substance prevents treeing. The positive 5 electrode is a body of lead, the article to be plated being connected with the negative wire. The electrolyte is at room temperature and is kept in agitation to insure a uniform deposition of the lead over the entire 10 surface of the article. A weak current should be used, that is, a current of not more than one ampere per square foot of surface to be plated which may be later increased to two amperes. If too strong a current is 15 used the plating will be spongy.

By this method the coating may be built up to any desired thickness and will be dense and have a smooth exterior surface. The original lead coating obtained through 20 chemical action in the first step of the process protects the iron from contact with the electrolyte, thereby preventing the chemical reaction between the iron and the electrolyte which would interfere with the 25 proper deposition of the lead on the iron if an attempt were made to deposit the lead directly on the iron surface by electrolytic action.

If it is desired to plate the article with 30 some other metal than lead, for example, with tin, copper, nickel or silver, the article after being lead coated in accordance with the first step of the method above described, that is, by immersion in the salt solution of 35 lead or in a bath of molten lead, will be electro-plated with copper, tin, nickel or silver, as the case may be, using any of the ordinary electro-plating methods common for these operations.

40 This application is a continuation in part of my copending application Serial No. 397,179 filed July 19, 1920 as a division of application Serial No. 374,089 filed April 15, 1920 (patented Jan. 31, 1922, as Patent 45 No. 1,405,167).

I claim:

1. Method of plating a metal article which consists in covering the article with a coating of lead, and then superposing on the 50 coating thus formed a second coating produced by electrolysis.

2. Method of plating a metal article which consists in covering the article with a coating of lead and then superposing on the 55 coating thus formed a second coating of lead produced by electrolysis.

3. Method of plating a metal article electro-positive to lead which consists in first bringing the article into contact with a solution of lead acetate to produce a deposition of lead on the article, and then superposing on the coating thus formed a second metal plating produced by electrolysis.

4. Method of plating a metal article electro-positive to lead which consists in first

bringing the article into contact with a solution of lead acetate to produce deposition of lead on the article, and then superposing on the coating thus formed a second lead coating produced by electrolysis. 76

5. Method of plating a metal article which consists in first bringing the article into contact with a water solution of a salt of a plating metal to produce deposition of the plating metal on the article, and then superposing on the first coating thus formed a second metal plating produced by electrolysis. 77

6. Method of plating which consists in first bringing the article into contact with 80 a solution of lead acetate having a concentration of at least 35% by weight, and then superposing on the lead coating thus formed a second coating produced by electrolysis.

7. Method of plating which consists in first bringing the article into contact with a solution of lead acetate having a concentration of at least 35% by weight and then superposing on the lead coating thus formed 85 a second lead coating produced by electrolysis. 90

8. Method of lead plating an iron or steel article which consists in first bringing the same into contact with a concentrated solution of lead acetate without electric current, then subjecting the article to an electro-plating operation using a lead salt solution of lesser concentration as an electrolyte. 95

9. Method of lead plating an iron or steel article which consists in first bringing the same into contact with a concentrated solution of lead acetate without electric current, then subjecting the article to an electro-plating operation using a lead salt solution of lesser concentration as an electrolyte, 100 and keeping the electrolyte in agitation. 105

10. Method of lead plating an iron or steel article which consists in first bringing the same into contact, without electric current, with a solution of lead acetate having a concentration of at least 35% by weight, and then subjecting the article to an electro-plating operation using a lead salt solution having a concentration of substantially 10% by weight. 110

11. Method of lead plating an iron or steel article which consists in first bringing the same into contact, without electric current, with a solution of lead acetate having a concentration of at least 35% by weight and then subjecting the article to an electro-plating operation using as an electrolyte a solution of lead acetate of substantially 10% concentration. 115

12. Method of lead plating an iron or steel article which consists in first bringing the same into contact, without electric current, with a solution of lead acetate having a concentration of at least 35% by weight and then subjecting the article to an electro- 120

130

plating operation using as an electrolyte a solution of lead acetate of substantially 10% concentration, and keeping the electrolyte in agitation.

5. 13. Method of lead plating an iron or steel article which consists in first bringing the same into contact, without electric current, with a solution of lead acetate having a concentration of at least 35% by weight, then subjecting the article to an electro-plating operation using as an electrolyte a solution of lead acetate of substantially 10% concentration, and keeping the electrolyte in agitation, employing for the electrolysis a current not in excess of one to two amperes per square foot of surface to be plated.
10. 14. Method of lead plating an iron or steel article which consists in first bringing

the same into contact, without electric current, with a solution of lead acetate having 20 a concentration of at least 35% by weight, then subjecting the article to an electro-plating operation using as an electrolyte a 25 solution of lead acetate of substantially 10% concentration, and keeping the electrolyte in agitation, employing for the electrolysis a current of substantially one ampere per square foot of surface to be plated which is increased during the electro-plating operation to two amperes per square foot. 30

15. A metal article covered with a dipped coating and an electrolytic coating, each consisting principally of lead and one coating superposed on the other.

ROBERT JAY SHOEMAKER.